

## UNITED STATES PATENT OFFICE

2,228,252

## EXTREME PRESSURE LUBRICANT

Henry G. Berger and Darwin E. Badertscher,  
Woodbury, and Francis M. Seger, Pitman, N. J.,  
assignors to Socony-Vacuum Oil Company, In-  
corporated, New York, N. Y., a corporation of  
New York

No Drawing. Original application December 3,  
1937, Serial No. 177,891. Divided and this ap-  
plication June 28, 1938, Serial No. 281,634

3 Claims. (Cl. 252—46)

This invention has to do in a general way with the art of lubrication and is more particularly concerned with the development of a lubricant composition adapted for use under extreme pressure conditions.

As is well known to those familiar with the art, the ordinary type of hydrocarbon lubricant, comprised only of a petroleum fraction, is incapable of withstanding the enormous pressures encountered between engaged surfaces in various types of modern machinery, such as the hypoid gears used in motor vehicles. This fact has led to the development of the so-called extreme pressure lubricant, which is comprised of a suitable carrying agent, such as a mineral oil, containing a minor proportion of an ingredient which, under the extreme pressure conditions encountered, will provide or form between the engaged surfaces a lubricating film capable of withstanding these high pressures. Ingredients of the type just referred to are known as extreme pressure ingredients or extreme pressure (E. P.) bases, and numerous materials have been proposed for such use. Among the various E. P. bases which have been proposed and which have met with varying degrees of success are organic materials which contain sulfur and chlorine. Our present invention is related to this general type of compound. This application is a division 30 of our copending application Serial No. 177,891, filed December 3, 1937.

It is a primary object of this invention to provide an extreme pressure lubricant which contains a new and novel sulfur-and-chlorine-containing material or compound capable of giving extreme pressure lubricant properties to a carrying agent such as a hydrocarbon lubricant oil otherwise incapable of withstanding extreme pressure conditions. In this regard we have discovered that perchloromethyl mercaptan and the class or group of compounds obtained by reacting various reactive materials with perchloromethyl mercaptan are very effective extreme pressure lubricant addition agents. The present invention is concerned specifically with the production of extreme pressure lubricants by the direct addition of perchloromethyl mercaptan to the oil. The various perchloromethyl mercaptan reaction products of the type mentioned above are described and claimed in our copending applications Serial Nos. 177,891 and 177,890, filed December 3, 1937.

Perchloromethyl mercaptan is a chlorinated substituted sulfur chloride having the formula  $\text{Cl}_3\text{C}-\text{SCl}$  and can be prepared by the chlorina-

tion of carbon disulfide according to the method of Heifrich and Reid (Jour. Amer. Chem. Soc. 43, 591 (1921)). For example, carbon disulfide containing about .4% by weight of iodine was chlorinated in the absence of direct sunlight at a temperature maintained below 25° C. until the volume of the reaction mixture had doubled. This crude reaction product, which contains carbon tetrachloride and sulfur chlorides in addition to perchloromethyl mercaptan, can be used in the preparation of the lubricants contemplated by this invention, but it is preferable to purify the crude product by distillation on a water bath at 100° C., followed by steam distillation. Subsequent vacuum distillation of the material refined in this manner indicated that the steam distilled material was practically pure.

To demonstrate the effectiveness of perchloromethyl mercaptan as an extreme pressure lubricant ingredient we have prepared and tested compositions comprised of a mineral oil to which perchloromethyl mercaptan has been added. More specifically, we have added a minor proportion of perchloromethyl mercaptan to a mineral oil having a Saybolt Universal Viscosity of 80 to 90 seconds at 210° F. and have subjected samples of such blended lubricants to the Almen Pin test, described by Wolf and Mougey, Proc. A. P. I., 1932, pages 118-130, and the S. A. E. test, described in S. A. E. Journal 39, 23-4 (1936).

These two tests are commonly accepted in the art as standards to determine the extreme pressure characteristics of a lubricant. In the table below we show typical results obtained with such tests, using the oil alone and a sample of the same oil blended with perchloromethyl mercaptan.

| Product                    | Percent<br>in oil | Almen   | Extreme Pres-<br>sure tests (lbs.<br>failed) S. A. E.<br>(1000 R. P. M.<br>14.8:1 rubbing<br>ratio, 8.35<br>lbs./sec. load-<br>ing rate |
|----------------------------|-------------------|---------|-----------------------------------------------------------------------------------------------------------------------------------------|
| Oil without addition agent |                   | 3,000   | <15                                                                                                                                     |
| Perchloromethyl mercaptan  | 1                 | 30,000+ | 410                                                                                                                                     |

From the foregoing example it will be seen that the perchloromethyl mercaptan or such perchloromethyl mercaptan condensation products as may be formed within the oil when the perchloromethyl mercaptan is added directly thereto, provide a highly efficient extreme pressure lubricant. The amount of perchloromethyl

5

10

15

20

25

30

35

40

45

50

55

mercaptan used may vary from say 0.1 per cent to 20 per cent, but in general lower percentages, say from 0.1 per cent to 10 per cent, are preferred.

- 5     Although we have indicated in the foregoing description that a mineral lubricating oil is a preferred carrying agent for the extreme pressure ingredients contemplated by our invention, it is not our intention that the invention be limited to any particular carrying or blending medium, but our invention includes broadly extreme pressure lubricants containing the perchloromethyl mercaptan described above, dissolved, dispersed, or emulsified in any other suitable carrying medium, such, for example, as fatty vegetable and animal oils; light petroleum hydrocarbons such as kerosene, etc., benzene and related hydrocarbons; alcohols, esters; ethers, etc.

We claim:

1. An extreme pressure lubricant comprising a hydrocarbon lubricant oil to which a minor proportion of perchloromethyl mercaptan has been added.
2. An extreme pressure lubricant comprising a hydrocarbon lubricant oil to which has been added a minor proportion of from about 0.1% to about 10% of perchloromethyl mercaptan.
3. An extreme pressure lubricant comprising a viscous mineral oil to which has been added about one percent of perchloromethyl mercaptan.

HENRY G. BERGER.

DARWIN E. BADERTSCHER. 15

FRANCIS M. SEGER.